

Jan. 13, 1959

A. MARZOCCHI ET AL

**2,868,669**

## METHOD OF CLEANING AND COATING SIZED GLASS FABRIC

Filed Sept. 2, 1954

2 Sheets-Sheet 1



**INVENTORS**  
**ALFRED MARZOCCHI**  
**REMUS F. CAROSELLI**  
**GERALD E. RAMMEL**  
**pv**

BY  
Haelin & Overman  
ATTYS.

Jan. 13, 1959

A. MARZOCCHI ET AL

2,868,669

METHOD OF CLEANING AND COATING SIZED GLASS FABRIC

Filed Sept. 2, 1954

2 Sheets-Sheet 2



INVENTORS  
ALFRED MARZOCCHI  
REMUS F. CAROSELLI  
GERALD E. RAMMEL  
BY

*Stacklin & Overman*  
ATTYS.

1

2,868,669

**METHOD OF CLEANING AND COATING SIZED  
GLASS FABRIC**

Alfred Marzocchi, Pawtucket, and Remus F. Caroselli, Manville, R. I., and Gerald E. Rammel, North Attleboro, Mass., assignors to Owens-Corning Fiberglas Corporation, a corporation of Delaware

Application September 2, 1954, Serial No. 453,782

6 Claims. (Cl. 117—46)

This invention relates to the treatment of fibrous glass and products thereof and particularly to improving the physical properties of fibrous glass in the form of fabric or the like.

In treating fabrics woven of fibrous glass in an attempt to color the glass, it has been found advantageous to heat clean the glass prior to dyeing or printing. Certain of the fabrics such as staple fabrics and the soft, thick satin weaves produced either from staple or continuous fibers have presented a problem when attempts have been made to heat clean them using the conventional equipment and methods. Heat cleaning of the fabrics has a dual purpose: (1) a fresh and clean surface which is highly receptive to chemical combination with treating substances is presented upon the fibers and strands, and (2) strands from which the fabric is woven become weave set.

Removal of the size or lubricant which was applied to the fibrous glass in order to facilitate forming and weaving is necessary in order to present clean glass surfaces to which the fabric finish can adhere. The fibers may be cleaned by washing; however, it has been found preferable to burn the size, lubricant and/or other treating material from the surfaces of the fibers in order to clean them. Controlling the heating of the fibrous glass is always a problem; however, when thick fabrics and staple fabrics are being treated, the problem is even more pronounced.

It is an object of this invention to provide improved methods for treating fibrous glass to improve the physical properties thereof.

It is a further object to provide a method and apparatus for heat cleaning, weave setting, and improving the drape of glass fabric.

Further objects will be apparent from the description of the invention which follows.

In the drawings, Figure 1a is a side elevation of part of the apparatus of the invention;

Figure 1b is a side elevation of the remainder of the apparatus;

Figure 2 is an enlarged side elevation of the feed end of the apparatus showing the scray pan and preheat roll; and

Figure 3 is a perspective view of the preheat roll.

The apparatus comprises a let-off stand 11, idler rolls 12, 12, a pair of pull rolls 13, 14, the former being driven and the latter being an idler. Idler roll 14 is adapted for movement through the horizontal plane into and out of contact with driven pull roll 13. The pull rolls are actuated when scray pan 15 is to be filled. Scray pan 15 is filled during lacing operations and when a splice is to be made between ends of fabric as when a new roll 16 is being placed on let-off stand 11. Roll 16 when supported in let-off stand 11 has a leather strap brake 17 which provides a constant resistance to unrolling of the fabric, see Figure 2. As seen in Figure 2, a sewing

2

machine 18 provided with a transverse railway carriage is mounted on frame 19 for securing the ends of rolls of fabric together.

Guide roll 21 is disposed above scray pan 15 as are the three tensioning rolls 22, 22. The uppermost tensioning roll is provided with a leather strap braking member 23. After the fabric passes over expander roll 24 where the longitudinal wrinkles in the cloth are removed, it passes around preheat roll 25 and then over guide rolls 26, 27 before entering weave set oven 28. The weave set oven is provided with a plurality of gas burners 29, 29, which heat the oven to the desired temperature. The combustion products from the burners surround a stainless steel muffle 31 in the oven 28 and are then vented through exhaust stack 32.

Stainless steel muffle 31 through which the fabric passes is provided with air manifolds 42, 42 which are adapted for directing air or oxygen upon the upper and lower surfaces of the fabric being heated, see Figure 1a. The two air manifolds are disposed one above the other and extend transversely across the width of the muffle and the fabric. The air manifolds 42, 42 have a plurality of openings which direct a stream of air or oxygen at a 45° angle toward the surface of the fabric being treated and against the direction of travel of the fabric as it passes through the muffle 31 of the weave set oven. Stainless steel muffle 31 is vented through exhaust stack 33 which is positioned above air manifolds 42, 42 and extends at its lower end across the width of stainless steel muffle 31. At the entrance and exit of the stainless steel muffle and of oven 28 are adjustable doors 34, 34 and 35, 35.

Above preheat roll 25 is an exhaust duct 36 adapted for removing gases given off by the fabric due to volatilization as the fabric passes over preheat roll 25.

As seen in Figure 3, preheat roll 25 comprises a large diameter roll having a smooth outer surface and an inner burner 37 comprising a pipe having a plurality of small openings 38, 38 through which gas-air mixture emits. Premixing chamber 39 is supplied with air and gas as indicated and the gas and air mixture is then supplied to both ends of the inner burner 37 by the piping system shown. Gas valve 41 controls the flow of gas and air mixture to inner burner 37. Heat cleaned fabric 43 passes over guide roll 44 as it emits from weave-set oven 28.

Draw roll unit 45 comprises two motor-driven rolls 46, 46 positioned one above the other and one idler roll 47. The draw roll unit pulls the fabric through the weave set oven with the proper tension, and also feeds the fabric into padder 48. Draw roll unit 45 is provided with a scray pan 49 which is used when the fabric is to be heat cleaned only. When heat cleaning only, the fabric is directed to a roll-up unit immediately after passing over the draw roll unit 45 and the scray pan is used when changing rolls at the roll-up unit.

Driven rolls 46, 46 may be rubber covered or may be stainless steel rolls which are water cooled to help resist the oxidation which normally takes place because of the elevated temperatures to which the draw roll unit is subjected.

Padder 48 comprises a guide roll 51, an immersion roll 52 disposed within dip pan 53, expander roll 54, and a pair of padder rolls 55, 55. The padder rolls are large diameter rubber covered rolls, the rubber having a shore "A" Durometer hardness of about 65. The lowermost padder roll is partially submerged in the liquor contained in tank 56. The uppermost padder roll is journaled in lever arms 57 which are pivoted at pivot point 58 and connected to air cylinders 59 through linkage 61. The lower padder roll is driven by an elec-

tric motor 62 and drive chain 63 and the upper padder is free to turn on its own axis.

The finishing agent, which may or not include a dye as applied by padder 48, is set by passing the treated fabric 64 through drying oven 65. The drying oven is provided with a plurality of chain driven rolls 66, 66 over which the fabric passes in the required number of passes as it is being dried. After the fabric leaves the drying oven, it is directed to roll-up unit 67. Roll 68 of the take-up section 69 is driven by electric motor 71 through drive belt 72. The spindle of roll-up stand 73 is driven by motor 74 through drive belt 75. A spray pan 70 is disposed between take-up section 69 and roll-up unit 67. Take-up section 69 runs at a constant speed and feeds the fabric to roll-up stand 73. During the time required to remove full rolls of the finished product, the fabric is deposited into spray pan 70. The speed of the roll-up stand 73 varies as the roll size increases as this section is driven by a constant torque motor.

Although only one padder and one drying oven are shown, for many applications another padder and oven is inserted into the line between the drying oven 65 and roll-up unit 67 shown in Figure 1b. Any number of padders or padders and ovens may be inserted as desired. Two, three or more successive padding and drying steps are sometimes used.

The production equipment as described has a central direct current (D. C.) controlled drive system for regulating the speed of the fabric from the draw roll unit 45 to the roll-up unit 67. Rheostats are located at the draw roll unit 45, the oven 65, the padder 48 and roll-up unit 67 to control the speed of the fabric so that the tension can be finely adjusted at each unit.

For the purposes of illustration and not intending to limit the invention thereto, a description of the treatment of a particular fabric will be described. A decorative fabric comprising fill yarns having a size thereon comprising the following ingredients in weight per cent is the starting material.

#### Example I

| Ingredient:                 | Percent by weight |
|-----------------------------|-------------------|
| Tricresyl phosphate         | 10.0              |
| Ethylene oxide polymer      | 5.0               |
| Alkylaryl polyether alcohol | 0.5               |
| Water                       | 84.5              |
|                             | 100.0             |

Ingredients which may be added to this forming size in addition to or as a substitute for the alkylaryl polyether alcohol are such materials as polyamines, tetraethyl pentamine, dibasic acids, a methyl ester of rosin, phenolic resins, polyvinyl methyl ether maleic anhydride, polybutenes, ethylene oxide-polyoxy propylene condensation products, titanium glycolates, titanium acylates, polyvinyl acetate, polyvinyl methylether, chlorinated alkanes, chlorinated petroleum waxes, and the like. The staple size comprises basically from 5 to 25% by weight tricresyl phosphate and from 5 to 25% ethylene oxide polymer, the remainder being water.

Other suitable sizes may be used for either or both the fill and warp yarns of the fabric; for instance, a carbon tetrachloride and kerosene mixture is entirely satisfactory as the size for the fabric to be treated. Mixtures of ethylene oxide polymer or other lubricants and water with no addition of tricresyl phosphate may be used as the size also.

The yarns from which the fabric is woven may be treated with a gelatine size such as is disclosed in U. S. Patents 2,245,620 and 2,371,933 issued to Hans Steinbach on June 17, 1941, and March 20, 1945, respectively.

Fabrics which have been successfully used are those having warp yarns treated with a size comprising gela-

tinge and an oil and fill yarns treated with the size of Example I.

In starting the apparatus a leader cloth constructed of fibrous glass and heavy glass cord are used. A wooden shell or tube of leader cloth is placed on let-off stand 11 and brake 17 is released. The leader cloth is laced through the apparatus substantially following the path shown in Figures 1a and 1b. Metal hooks or the like are used to pull the leader cloth through weave set oven 28. After the leader cloth is laced through draw roll unit 45, heavy glass cords which have been laced through the padder rolls 55, 55, drying oven 65, and roll-up unit 67 are secured to the leader cloth.

Once sufficient leader cloth has been taken through the charge end of the line, a roll of fabric to be treated is placed on the let-off stand and the cloth end is attached to the end of the leader cloth by using sewing machine 18. A single stitch seam using glass sewing thread is made.

After the lacing has been completed, weave set oven 28 and drying oven 65 are brought to operating temperature by lighting the gas burners in each. Gas valve 41 is opened and preheat roll 25 is lighted to bring the preheat roll up to operating temperature. The preheat roll may be maintained at a temperature of from 500° to 900° F. when processing a fabric at least some of the yarns of which have a forming size thereon such as that described in Example I, a surface temperature of 600° F. is preferred. The temperature of the weave set oven 28 may be from about 900° to 1300° F. A temperature of 1200° F. is preferred when a staple yarn fabric comprising fill yarns having the size of Example I and warp yarns with gelatine size is being treated. A staple fabric comprising 100% staple fibers treated with the size of Example I is fully heat cleaned at a temperature of about 1000° F. Drying oven 65 is maintained at a temperature of from 200° to 400° F. and preferably from 275° to 375° F. The drying oven temperature is preferably about 360° F.

The finish or after treatment solutions are prepared and introduced into dip pan 53 and adjoining tank 56.

A finish comprising the following ingredients is prepared and introduced into both dip pan 53 and tank 56.

#### Example II

| Ingredient:                                                                              | Percentage by weight |
|------------------------------------------------------------------------------------------|----------------------|
| Polyvinyl alcohol (98% hydrolyzed)                                                       | 1.5                  |
| Quaternary nitrogen compound (reaction product of an amide reacted with triethanolamine) | 8                    |
| Stearo chromic chloride                                                                  | 2                    |
| Water                                                                                    | 88.5                 |

As the process continues more finish is added to dip pan 53 as required to replace that being applied to the fabric. Other suitable finishes include those of U. S. Patent 2,686,737, issued August 17, 1954. Pigments and dyestuffs are added to the finish when desired.

The central drive is energized and the process is then commenced. The fabric to be treated is advanced through weave set oven 28 by the action of draw roll unit 45. As the fabric passes over preheat roll 25, volatile gases from the size on the fabric are driven off. The volatile gases from the tricresyl phosphate and ethylene oxide are removed through duct 36. The fabric then passes horizontally through weave set oven 28 where the size is first carbonized and then completely burned off leaving a white cloth comprising fibers having clean surfaces. When the fabric passes air manifolds 42, 42, the combustion of the size is completed. Complete combustion of the size is indicated when a blue colored flame is produced in the weave set oven. The jets of air or oxygen from manifolds 42, 42 preferably are directed at a 45° angle toward the oncoming fabric. Complete combustion of the size materials upon the fabric will make it possible to achieve

a true white fabric. Then if the fabric is to be dyed, true color shades can be accomplished or if the fabric is to remain undyed, a true white is provided.

When using the preferred temperatures, the fabric is advanced at a rate of 18½ feet per minute. Air cylinders 59 are set so that the pressure on the padder rolls 55, 55 is 35 pounds per square inch. In the padder unit the fabric is drawn through dip pan 53 and then through padder rolls 55, 55 which distributes the finishing agent throughout the fabric and removes the excess finish. The excess finish is collected in tank 56 and is returned to dip pan 53 through a connecting tube. The tension of the fabric between the draw roll unit 45 and padder 48 is controlled by adjusting the speed of the padder rolls 55, 55 with a rheostat which is a part of the D. C. central drive system.

As the fabric travels through drying oven 65 moisture is removed from the finish on the fabric and the finish becomes set upon the fabric.

When treating staple fabrics and satin weave fabrics and the like, it is necessary to use a preheat roll such as that disclosed in order to control the cleaning of the fabric in the weave set oven. The volume of volatile gases which are driven off within the weave set oven if no preheat roll is used is great enough when treating these fabrics that it is very difficult and at times impossible to control the temperatures attained in the weave set oven. It has been discovered that by using a preheat roll the volatiles can be driven off controllably and that the remainder of the size is then burned off with a greater degree of accuracy and complete combustion can be attained without destruction of the physical properties of the fibrous glass.

When running fabrics such as staple fabrics, the pull rolls are usually maintained open. When treating such fabrics, draw roll unit 45 pulls the fabric through the weave set oven. When the need for a new roll arises, pull roll 14 is moved into contact with pull roll 13 and pull rolls 13 and 14 are speeded up to accumulate enough fabric in the scray pan 15 to allow time for the splicing operation. When the splice has been made, pull roll 14 is again moved to the open position and driven roll 13 is stopped. When treating other fabrics such as marquisette, pull rolls 13 and 14 are maintained in a closed or in-contact position except when a splice is being made. A supply of fabric is maintained in the scray pan 15 at all times, the amount being controlled by adjusting the speed of the pull rolls 13, 14. Heavy fabrics such as casement fabrics, staple fabrics and the like are not folded in the scray pan 15 except when it is necessary to make a splice.

As stated before, more than one padder and drying oven may be used. Two padders and two drying ovens are used when applying finishes comprising butadiene acrylonitrile and stearato chromyl chloride or tetrafluoroethylene or polyethyl acrylate and colloidal silica and the like. For instance, when applying a finish comprising polyethyl acrylate and stearato chromyl chloride, the following procedure is followed.

The fabric is passed through the weave set oven which is maintained at a temperature of from 1150° F. to 1225° F. at a speed of about 20 feet per minute. The fabric passes through the first padder where an emulsion of polyethylacrylate and dye is applied and then the fabric is dried at a temperature of from 275° to 300° F. A dispersion of stearato chromyl chloride is applied at the second padder and the fabric is dried at a temperature of about 345° F.

The speed of the fabric through the apparatus may vary widely depending upon the type of fabric being treated and upon the size which has been applied to the fabric prior to its treatment in the apparatus of this invention. The speeds may vary from about 15 to about 80 feet per minute. The weave set oven temperatures vary also depending upon the speed at which the fabric is passed through the oven. If the speed of the fabric is increased,

the temperature of the weave set oven and the preheat roll are generally increased.

If desirable, the fabric may be passed through a vapor chamber to help remove wrinkles from the fabric; however, the preheat roll is very effective as a device to remove wrinkles.

It is possible using the apparatus of this invention to control the heat cleaning, weave setting and subsequent application of finishes and dyes with much greater accuracy. Higher quality products are possible because of this added control. Complete cleaning allows perfectly white fabrics to be produced and, in addition, gives brighter and truer shades of color when the finish includes a dye. In addition to these advantages, certain of the heavy fabrics including the staple fabrics are now treated under controlled conditions. The continuous two-step heating process carried out by the preheat roll and the weave set oven has provided the key to treatment of heavy bulky fabrics such as staple fabrics and the like.

Various modifications can be made within the spirit and scope of the following claims.

We claim:

1. Method of applying a finish to a fibrous glass fabric having a size thereon comprising a two-stage cleaning step and a finish application step, said two-stage cleaning step

25 comprising advancing said fabric toward a combustion chamber, heating said fabric immediately prior to its reaching said combustion chamber to a temperature of from about 500° to 900° F. to drive off sufficient amount of the size in the form of volatile materials to allow controlled heat cleaning of the fabric in a subsequent step but leaving sufficient amount of size thereon to allow burning of the remaining size to provide complete heat cleaning, and then heating said fabric in a combustion chamber to

30 a temperature of from about 900° to 1300° F. while simultaneously directing a stream of a combustion supporting gas toward the surfaces of said advancing fabric to heat clean and weave set the fabric.

2. Method of cleaning fibrous glass fabric having a size thereon comprising continuously advancing the fabric toward an oven having a combustion chamber, heating said advancing fabric while it is outside the combustion chamber to a temperature at which a sufficient portion of the size in the form of volatile materials will be removed from the fabric to allow controlled heat cleaning by burning in a subsequent step, and heating the fabric within the combustion chamber to a temperature sufficient to burn completely all materials remaining on the fabric to provide a completely cleaned fabric.

3. Method of claim 2 wherein the fabric is heated to a temperature of from about 500° to about 900° F. outside the combustion chamber.

4. Method of claim 3 wherein the fabric is heated to a temperature of from about 900° to about 1300° F. within the combustion chamber.

5. Method of heat cleaning heavy fabrics of glass having a size thereon comprising heating the fabric to remove a sufficient portion of the size in the form of volatile materials to allow controlled and complete removal of remaining portions of the size in a subsequent burning step, and heating the fabric to a temperature of from about 900° to about 1300° F. in a combustion chamber for complete heat cleaning.

6. In a process of heat cleaning fibrous glass fabric having a size thereon comprising heating the fabric in a combustion chamber to a heat cleaning temperature of from about 900° to about 1300° F., the step of heating the fabric prior to introduction into the combustion chamber to a temperature sufficient to remove a portion of the size in the form of volatile materials from the fabric so that the above heat cleaning temperature range can be maintained within the combustion chamber for complete heat cleaning by burning.

**References Cited in the file of this patent**  
**UNITED STATES PATENTS**

|           |         |               |
|-----------|---------|---------------|
| 790,050   | Hall    | May 16, 1905  |
| 1,863,687 | Cramer  | June 21, 1932 |
| 1,940,975 | Shaver  | Dec. 26, 1933 |
| 2,344,601 | Collins | Mar. 21, 1944 |

|           |        |               |
|-----------|--------|---------------|
| 2,633,428 | Klug   | Mar. 31, 1953 |
| 2,667,568 | Ferier | Jan. 26, 1954 |

**OTHER REFERENCES**

Coronizing Process Manual, publ. by Owens-Corning Fiberglas Corp., N. Y., 1948, pp. BA-1 to 3; BB-1; CA-2; CE4 and CE5.